

## UNITED STATES PATENT OFFICE

2,186,245

## ELECTRICAL CONTACT MEMBER

James M. Kelly, Trafford, Pa., assignor to Westinghouse Electric & Manufacturing Company, East Pittsburgh, Pa., a corporation of Pennsylvania

No Drawing. Application May 5, 1939,  
Serial No. 271,934

## 5 Claims. (CL 200—166)

This invention relates to electrical make and break contact members.

Contacts formed from refractory metal powders and a metal having good conductivity, such as copper or silver, have been employed heretofore. Such metals having high conductivity, are, however, not of themselves entirely satisfactory for this purpose, since the resulting contact member does not have as high physical properties as are required in certain applications.

Carbon has been so added to the composition of the contact members that when heat treated it will combine with the refractory metal and form a refractory carbide, thereby increasing the hardness of the contact members. Such refractory carbides are undesirable in the contact members since they increase the resistivity of the metal and lower the melting point of the refractory with which the carbon combines.

Other alloying metals have been added in addition to the copper or silver in making the contact member in an effort to enhance the physical properties of the resulting contact member, but such additions have the disadvantage that they affect the oxidation rate of the contact members and introduce impurities therein without appreciably increasing the physical properties of the contact member. Further, where some of these alloying metals have been utilized, it has been found that a satisfactory bond is not perfected between the refractory metal and the alloying metals, it being difficult to secure a satisfactory wetting action of the alloy with refractory metal.

An object of this invention is to provide a contact member having high physical properties and good wear characteristics.

Another object of this invention is to provide a composite contact member formed from refractory metal powders and a silver base alloy containing copper and antimony.

A further object of this invention is to provide a contact member formed from refractory metal powders and a silver base alloy containing copper and antimony, and which is susceptible to an age-hardening heat treatment to improve the mechanical strength of the contact member.

Other objects of this invention will become apparent from the following description and the appended claims.

In practicing this invention, a contact member is formed from a plurality of metals which have been found to cooperate to give certain desired characteristics. A base body of refractory metal selected from the group consisting of tungsten and molybdenum, and which has a relatively high

melting point so formed as to have interstices therein, and which of itself does not possess the desired mechanical strength, is impregnated with a silver base alloy of lower melting point, as will be disclosed more fully hereinafter.

In forming the metal base here employed, refractory metal powders of predetermined size ranging from 150 to 250 mesh are mixed with sufficient organic bond to form a plastic putty-like mass which is moldable, or which can be rolled or cast to a desired shape. Any suitable organic bond which can be removed by drying or sintering the shaped mass to leave a porous structure may be employed. It is desirable to employ a bond which can be substantially completely removed so as not to leave a carbon residue which may combine with the refractory metal in the form of a carbide, since such carbides are undesirable. An organic bond composed of about 75% of shellac and 25% of alcohol is entirely satisfactory in forming the putty-like mass, and when the mass is heated at a temperature of about 1000° C. to 1100° C. in a reducing atmosphere, it is substantially completely removed, leaving the desired porous structure.

In order to impart the desired characteristics to the contact member, the porous refractory metal base or body is then filled with the impregnating silver base alloy. The alloy employed in forming the contact members of this invention is a silver base alloy which contains between 1% and 10% of each of the alloying elements, copper and antimony. It is desired that at least 1% of each of copper and antimony be present in the silver base, since lower contents of copper and antimony are not effective for imparting the desired strength to the alloy and consequently to the resulting contact member impregnated with the silver base alloy.

In practice, it is found that a silver base alloy containing about 7.5% of copper and about 8% of antimony is effective in producing the desired mechanical strength in the resulting alloy. For practical purposes, however, it is found that a silver base alloy containing an optimum composition of from 3.5% to 4% of each of copper and antimony is satisfactory for the purpose of this invention, since comparable strengths are obtained as in the contact members impregnated with the silver base alloy having larger contents of the alloying elements, copper and antimony. It is thought that this is because copper and antimony in excess of about 4% in the silver base of the alloy does not go into solution in the silver base.

The silver base alloy employed in forming the contact member of this invention is susceptible to precipitation hardening, and when heat treated, as by quenching at from a temperature of between 600° C. and 775° C., and aged at a temperature of between 100° C. and 400° C., has a hardness greater than 70 Rockwell B. The same effect is found when a contact member formed of the refractory metal powders and impregnated with the silver base alloy containing copper and antimony is subjected to a similar heat treatment, giving a contact member having high mechanical strength.

In forming the contact members, from 45% to 15 75% by weight of the refractory metal powders is impregnated with from 55% to 25% by weight of the silver base alloy containing between 1% and 10% of each of copper and antimony. In impregnating the refractory metal powders, it is 20 found that, in addition to imparting strength to the alloy, the antimony constituent of the silver base alloy aids in securing a bond between the refractory metal powders and the impregnating alloy. It is thought that the antimony in the 25 silver base alloy acts as a fluxing agent, promoting and so accelerating the wetting characteristics of the silver base alloy that it readily impregnates the porous refractory structure, giving a contact member having a uniform structure in 30 which the refractory metal is securely bonded by the silver base alloy. Such contact members are resistant to corrosion, and when precipitation hardened, as hereinbefore described, have high physical properties, that is, high hardness, high 35 tensile strength, and resistance to wear or deformation.

A particular contact member formed in accordance with this invention, and which is satisfactory for use where it is desired to interrupt 40 heavy currents, is formed from about 60% of molybdenum powders impregnated with about 40% of the silver base alloy which contains about 4% of each of the alloying elements, copper and antimony. As quenched from 700° C., this contact 45 member has a Rockwell B harness of 20, whereas when aged for only 10 hours at 200° C., the hardness and consequently the strength of the resulting contact member is increased to a Rockwell B hardness of 71. The resulting contact 50 member is particularly resistant to corrosion and has a long life when measured in terms of interrupting operations.

By practicing this invention, contact members are produced having good mechanical strength, 55 and which are free from carbon contaminations

sometimes employed heretofore for improving the wearing characteristics of the contact members. With the combination of metals employed, a contact member is produced which can readily be machined to shape prior to the described precipitation hardening treatment, and which afterwards can be heat treated to render them resistant to deformation when subjected to repeated blows such as are encountered in service. A micro-examination of the contact members embodying the teachings of this invention reveals 10 that the silver base alloy containing copper and antimony is distributed very uniformly throughout the matrix of refractory metal in a very finely divided state of subdivision. Such contact 15 members are resistant to corrosion and can be utilized in service where it is necessary to interrupt heavy currents without danger of contact failure.

Although this invention has been described 20 with reference to a particular embodiment thereof, it is, of course, not to be limited thereto except insofar as is necessary in accordance with the teachings of the prior art and the scope of the appended claims.

I claim as my invention:

1. An electrical contact member comprising from 45% to 75% by weight of refractory metal powders bonded together with from 55% to 25% of a silver base alloy containing from 1% to 10% of copper and 1% to 10% of antimony.

2. An electrical contact member comprising from 45% to 75% by weight of refractory metal powders formed to a predetermined shape and impregnated with a silver base alloy having a 35 copper content of from 1% to 10% by weight and an antimony content of from 1% to 10% by weight, and which has been precipitation hardened subsequent to the impregnation.

3. An electrical contact member comprising 40 about 60% of molybdenum and about 40% of a silver base alloy which contains between 1% and 10% of each of copper and antimony.

4. An electrical contact member as in claim 1 which has been quenched from a temperature of 45 between 600° C. and 775° C. and aged at a temperature of between 100° C. and 400° C.

5. An electrical contact member comprising a major proportion of refractory metal powders bonded together with a minor proportion of a 50 silver base alloy which contains from 1% to 4% of each of the allowing elements copper and antimony.

JAMES M. KELLY.